

# United States Patent [19]

[11] 3,793,823

Tallman

[45] Feb. 26, 1974

[54] **METHOD OF MAKING COMPLIANT SUSPENSION CABLE**

[75] Inventor: Charles V. Tallman, Rye Beach, N.H.

[73] Assignee: The United States of America as represented by the Secretary of the Navy, Washington, D.C.

[22] Filed: July 26, 1972

[21] Appl. No.: 275,128

## Related U.S. Application Data

[62] Division of Ser. No. 37,074, May 14, 1970, Pat. No. 3,696,325.

[52] U.S. Cl. .... 57/163

[51] Int. Cl. .... D02j 1/06

[58] Field of Search.... 57/6, 13, 15, 16, 17, 18, 36, 57/55.5, 139, 140 R, 144, 146, 152, 157 R, 157 S, 160, 163, 168; 139/423; 340/2

## References Cited

### UNITED STATES PATENTS

2,300,241 10/1942 Van Hoorhis..... 57/152 X

|           |         |                    |          |
|-----------|---------|--------------------|----------|
| 3,048,078 | 8/1962  | Kaplan.....        | 57/163 X |
| 2,017,444 | 10/1935 | Page .....         | 57/163 X |
| 3,540,493 | 11/1970 | Tallman.....       | 139/423  |
| 3,541,498 | 11/1970 | Dale et al. ....   | 340/2    |
| 3,543,228 | 11/1970 | Farmer et al. .... | 340/2    |

## FOREIGN PATENTS OR APPLICATIONS

475,399 11/1937 Great Britain ..... 57/152

Primary Examiner—Donald E. Watkins  
Attorney, Agent, or Firm—R. S. Sciascia; Henry Hansen

## [57] ABSTRACT

Compliant, nonstrumming, high strength composite cable and method of making thereof for a sonobuoy suspension system. Nonabsorbent relatively inelastic strands of textile yarn are bound onto an elastomeric warp strand by two counter wound helixes of textile stretch yarn. The inelastic yarn forms random transverse loops along the cable by protruding outwardly through the openings between the helical windings.

4 Claims, 3 Drawing Figures





## METHOD OF MAKING COMPLIANT SUSPENSION CABLE

### CROSS-REFERENCES TO RELATED APPLICATIONS

This is a division of application Ser. No. 37,074 filed May 14, 1970, now U. S. Pat. No. 3,696,325 issued Oct. 3, 1972.

### STATEMENT OF GOVERNMENT INTEREST

The invention described herein may be manufactured and used by or for the Government of the United States of America for governmental purposes without the payment of any royalties thereon or therefor.

### BACKGROUND OF THE INVENTION

The invention relates in general to a method of making composite suspension cables and more particularly to a method of making a new and improved composite elastic cables for underwater use having antistrumming fringe and at least one relatively inelastic longitudinal strand.

Underwater listening or sonar systems often employ remote sonobuoy stations having hydrophones or transducers suspended from a buoyant float containing transmitter or receiver. Suspension cables for the transducers are commonly made of compliant or elastic material to maintain the transducer at a fixed vertical level regardless of the frequently erratic movement imparted to the float by wave action on the surface. In addition, transverse ocean currents relative to a submerged vertical cable induce natural vibration or strumming of the cable causing vertical oscillation of the load. Compliance enhances the strumming effect, and if the load is a sensitive hydrophone, the spurious noise thus contributed to the background level may obscure a target signal.

One type of prior art antistrumming cable is shown in an application entitled "Improved Hydrophone Suspension Cable" by Charles V. Tallman, Ser. No. 803,763, filed Mar. 3, 1969, now U. S. Pat. No. 3,540,493 issued Nov. 17, 1970. The larger, woven cable, while ideal for use with relatively heavy loads, did not address itself to the special problems encountered with very light loads of a few ounces. Loads on this order are achieved even with massive transducer assemblies by incorporating buoyant material to reduce their weight in water. The load reduction, however, demands a similar decrease in the size and spring constant of the cable. On the other hand, towing of the sonobuoy or extremely rough sea may place abnormally high, transient stress on the cable. Thus, the suspension cable must be reliably operable over a wide range of tension, from a few ounces to several pounds or more.

All of the prior art cables which provide antistrumming fringe have numerous woven or braided elements requiring expensive machinery for fabrication. Usually the limit or break strength is determined solely by the strength of the compliant core. As a result, many of the prior art cables cannot be scaled down to yield the desired compliance for light loads without lowering their break strength below acceptable levels.

### SUMMARY OF THE INVENTION

Accordingly one of the principal objects of the invention is to provide a method for making a compliant,

high-strength suspension cable for suppressing noise generated by strumming. Another object of the invention is to provide a method for making a nonwoven elastic suspension cable of low spring constant of increased ratio of break strength to design load.

### BRIEF DESCRIPTION OF THE DRAWING

FIG. 1 is an elevation view of a sonobuoy deployed in water with a suspension cable made according to the invention;

FIG. 2 is an enlarged view of the cable of FIG. 1; and

FIG. 3 is an enlarged view of the cable of FIG. 1 fully stretched.

15

### DESCRIPTION OF THE PREFERRED EMBODIMENT

A sonobuoy is shown in FIG. 1 having a piezoelectric transducer assembly 10 suspended by a compliant cable 11 from a buoyant cylindrical float 12 which carries an amplifier and R.F. transmitter (not shown) and a whip antenna 13. If the sonobuoy is active rather than passive, that is, noise is to be generated rather than received by transducer 10, the transmitter will be replaced by an R.F. receiver enabling remote control of the transducer output. Electrical connection between float 12 and transducer 10 is provided by wire 14 which forms an open, loosely wound helix surrounding cable 11. The diameter of the helix greatly exceeds that of cable 11 to prevent interference. The sea water itself may be used for the grounded side of the electrical circuit.

The improved suspension cable 11 shown in more detail in FIG. 2 includes a relatively inelastic strand bundle 16 bound to an elastic warp element 17 by means of mesh-forming cover threads 18 and 19 which are wrapped on the cable in counterwound helixes having non-uniform pitch. In the larger open areas between cover threads 18 and 19, inelastic strands 16 protrude laterally to form intermittent loops 21. Between loops 21 threads 18 and 19 pass over the strand bundle 16 securing it to the elastic warp element. Due to the non-uniform helical pitch in threads 18 and 19, the loops occur at random intervals and serve as antistrumming fringe for noise suppression.

Warp element 17 is made from an elastic material such as a high-stretch, highly resilient synthetic rubber. Preferably, the warp material should be extensible to at least six times its unstretched length without exceeding its elastic limit. A preferred material for the warp element is 20 gauge, isoprene-polybutadiene blend synthetic rubber having a square cross section. The spring constant may be varied as desired for different loads by increasing the gauge or cross-sectional area of the elastic warp element or by using a plurality of such elements. Other synthetic rubbers, elastomers and elastic materials can be used depending on the stress-strain and frequency levels sought.

Multiple strands 16 which form the loops 21 are made of a nonabsorbent textile yarn such as 840 denier 6-turn twist polypropylene or polyester. The stress of the design load will be carried exclusively by elastic warp element 17. However at full extension, multiple strands 16 will be taut and loops 21 will no longer be present. At this point substantially all of the load will be borne by strands 16 which are made of relatively inelastic fibers. The number and denier of strands 16 may

be varied depending on the loop density and strength desired. Six strands have been found suitable for a four ounce load. The break strength of the composite cable is determined by the summated strength of the strands 16.

The helically wound cover threads 18 and 19 are preferably made of textile stretch yarn. Any overload on the cable will thus be borne entirely by the stronger inelastic yarns in the strand bundle 16. A yarn found suitable for this purpose is 70 denier Helanca nylon which reaches its limit of stretch at about 50 percent. However other low denier elastic fibers may be substituted for the cover threads.

One method of making the suspension cable 11 of FIG. 2 is to prestretch elastic warp element 17 and bind the straight strand bundle 16 thereto by wrapping cover threads 18 and 19 in counterwound helices of uniform pitch as shown in FIG. 3. When the tension is released, strand bundle 16 pushes through the openings between cover threads 18 and 19 at random intervals to form loops 21 in cable 11, illustrated in FIG. 2 under normal load conditions. As the elastomer 17 contracts, slack is introduced into strand bundle 16. The original uniform winding pattern is distorted as threads 18 and 19 are forced apart at various points along the length of the cable. The number of turns between any two resulting loops 21 may vary from one to five or more depending on the bunching or decreased pitch between loops 21 caused by the spreading of threads 18 and 19. The exact spacing between any two loops is noncritical. The original pitch on the wrapping helices is also noncritical and may be adjusted to give the composite texture sought. Typically, the cable might have 80 turns per foot when fully stretched.

Alternatively, cover threads 18 and 19 may be wound initially in helices having a regularly varying pitch. In this way, the position of loops 21 after relaxation may be predetermined, if desired.

In manufacture, the stretched element 17 and strand bundle 16 are juxtaposed and passed concurrently up through two counterrotating spindles. As the elements pass through each spindle, a helix of textile stretch yarns 18 and 19 is wound around the bundle of strands 16 and the elastic warp element 17. Tension on wrapping yarns 18 and 19 is regulated by flier or ring traveler constraints. Since the pitch of each helix is to remain uniform, the elements to be wrapped are fed through the spindle area at constant speed. The spindle rotation speeds also remain constant. State-of-the-art rubber covering machines encompass the needed speed ratios and spindle bores determined with reference to the denier of the wrapping threads 18 and 19 and the desired pitch or number of turns per inch thereof. The initial tension on the elastic warp element 17 may range approximately from 200 to 600 percent. The higher the initial stretch, the coarser side loops 21 will be. A suitable initial stretch has been determined to be about 380 percent.

An important advantage of the invention is the elimination of the complex machinery formerly necessary to form and maintain side loops or fringe on the suspension cable. In the manufacturing stage of the cable, no loops are present to interfere with the assembling of the constituent elements of the cable. The final stage of manufacture is automatically completed by releasing tension on the cable. The self-deploying loops 21 automatically distribute themselves in random fashion se-

lecting appropriate areas for protrusion and spreading of cover threads 18 and 19. Moreover, manufacture does not require weaving on a fabric loom and can be conveniently performed on conventional equipment.

The parameters of the improved cable 11 may be varied according to specific design criteria in a manner familiar to those skilled in the art. The spring constant of a given embodiment of the cable according to the invention is not strictly constant over its elastic range and increases as increased tension causes the cable's length to approach the limit of elongation. As a result, compliance may be reduced below the acceptable level. Thus, for heavier loads the diameter of the cable may have to be increased. The amount of tension produced under water by a given mass may be reduced by providing a determined amount of buoyancy within the load.

If the sonobuoy employs a passive hydrophone responsive to a selected bandwidth, the dimensions of the cable can be adjusted to obtain a natural, undamped strumming frequency outside of the selected bandwidth. Antistrumming loops 21 will still be needed, however, since some of the harmonics and associated frequencies may lie within the bandwidth.

There are many different means for the electrical connection between transducer 10 and float 12. For example, instead of a loose helix, wire 14 may form a series of open loops attached at relatively long intervals to cable 11. Alternatively, electrically conductive fibers may be used in strand bundle 16. If the diameter of the warp element 11 permits, wire 14 may be slidably carried within a central bore in element 17. However, some means of eliminating slack in the wire would be necessary, such as a tension-maintaining spool located in float 12.

Besides manufacturing convenience, the invention provides a new cable having an increased break-strength-to-load ratio, typically about 140, far in excess of that achieved by prior art compliant cables. The combination of an antistrumming fringe or loope network with high break strength in a miniature elastic cable is believed to be unprecedented. The new cable also meets the critical size and weight limitations dictated by available storage space and pay out mechanisms, especially where transducer depths of several hundred feet are desired.

It will be understood that various changes in the details, materials, steps and arrangements of parts, which have been herein described and illustrated in order to explain the nature of the invention, may be made by those skilled in the art within the principle and scope of the invention as expressed in the appended claims.

What is claimed is:

1. A method of making a suspension cable comprising the steps of:

stretching an elastic element and a first strand to the same length, the unstretched length of said element being shorter than the unstretched length of said first strand; and

helically winding a second strand around said element and said first strand.

2. A method according to claim 1 further comprising the step of:

helically counterwinding a third strand around said element and said first and second strands.

3. A method according to claim 2 wherein:

said second and third strands are wound in uniform pitch having a predetermined spacing between adjacent cycles of each helix, and spacing is sufficient to allow said first strand to protrude in loops at intermittent points through said second and third strands when unstretched. 5

4. A method according to claim 3 wherein:

said element is made of synthetic rubber;  
said first strand is made of relatively inelastic textile  
yarn; and  
said second and third strands are made of textile  
stretch yarns.

\* \* \* \* \*

10

15

20

25

30

35

40

45

50

55

60

65